

April 1, 1930.

D. FRIEDLÄNDER

1,752,665

PROCESS FOR THE MANUFACTURE OF SENSITIZED VELVET  
PAPER FOR PHOTOGRAPHICAL USES  
Filed July 7, 1927



*Inventor.*

Daniel Friedländer

*by C. S. Gogel*

*his Attorney.*

## UNITED STATES PATENT OFFICE

DANIEL FRIEDLÄNDER, OF BRUSSELS, BELGIUM, ASSIGNOR TO MESSRS. A. MEURSING AND E. J. GRATAMA, BOTH OF AMSTERDAM, NETHERLANDS

PROCESS FOR THE MANUFACTURE OF SENSITIZED VELVET PAPER FOR PHOTOGRAPHICAL USES

Application filed July 7, 1927, Serial No. 204,152, and in Germany July 7, 1926.

It has long been desired in the photographic industry, especially for portraits, to produce a paper with a dull surface giving the image a distinctly artistic character.

5 Salt paper without addition of gelatine, papers prepared with starch or the like and gelatine emulsion, Fresson paper, Bühler and Höchheimer papers and the like only half fulfill this object.

10 Therefore this invention has relation not to the sensitive coating but to its support. The velvet-like appearance must be obtained by the support. The paper must really possess a velvety surface, and not only the appearance.

15 Trials have proved that it is not sufficient to mix the coating with a vegetable or animal fibrous-dust, whereby said dust is embodied in the coating. A uniform distribution of the sensitized dust-fibres on the support would be nearly impossible without an adhesive medium; however, when adding an adhesive medium, the manufactured paper loses its velvet-like character, since the sensitized coating no longer consists in loose fibres.

20 25 Also the adhesive medium has for result to make the image flat i. e. lacking in depth.

This invention contemplates sensitizing the ready made velvet paper. Adhesive medium can then be dispensed with.

30 I am aware velvet papers have been known before, for instance as tapestries, drawing papers and the like. Same have been manufactured by spreading and fixing by an adhesive medium a vegetable or animal dust or

35 the like substance upon a paper.

35 In the accompanying drawing, the single figure, which illustrates a top plan view of my improved paper with a portion broken away, the well sized paper 10 is laid over with an adhesive medium 11 hardly soluble in water and the surface is spread over with a fibrous dust 12, such as fine white wool-powder. After complete drying, the excess of dust is brushed off with a soft brush and

45 the thus prepared paper is then sensitized.

I claim:

The process of making sensitized velvet paper for photographic use consisting in coating a well-sized sheet of paper with an adhesive material that does not readily dis-

solve in water then spreading over the surface a fine fibrous organic dust, drying the aforesaid material and removing the excess dust and finally sensitizing the paper over the dull velvety surface thus produced.

55 In testimony that I claim the foregoing as my invention, I have signed my name hereto.

DR. DANIEL FRIEDLÄNDER.

60

65

70

75

80

85

90

95